

June 9, 1942.

S. B. TUWINER ET AL

2,285,762

ELECTRODEPOSITION OF COPPER POWDER

Filed Feb. 4, 1938

2 Sheets-Sheet 1



INVENTORS  
and  
Sidney B. Tuwiner  
William H. Osborn  
By Paul R. Ames  
ATTORNEY

June 9, 1942.

S. B. TUWINER ET AL

2,285,762

ELECTRODEPOSITION OF COPPER POWDER

Filed Feb. 4, 1938.

2 Sheets-Sheet 2

Fig. 3



Fig. 4



Fig. 5



Fig. 6



Fig. 7



Fig. 8.



Inventors  
Sidney B. Tuwiner  
and William H. Osborn  
By Paul R. Ames  
Attorney

## UNITED STATES PATENT OFFICE

2,285,762

## ELECTRODEPOSITION OF COPPER POWDER

Sidney B. Tuwiner, Kew Gardens, and William H. Osborn, New York, N. Y., assignors to Phelps Dodge Corporation, New York, N. Y., a corporation of New York

Application February 4, 1938, Serial No. 188,770

12 Claims. (Cl. 204—10)

This invention relates to the preparation of copper and particularly to the electrodeposition of copper in flake form.

Copper powder is used as a pigment ingredient in the most durable types of paint for the coating of steel and wood in manufacturing plant maintenance, for antifouling paints, under-water ship hull paints and for other marine paints. Such paints, including air-drying varnish vehicles, have the property of retaining a certain degree of plasticity or "life," thereby resisting the embrittling effect of prolonged weathering, which causes many other types of paint to fail by checking, cracking and flaking. Copper paints have been shown to be excellent for prime coats as well as for overcoats for metal painting.

Copper is also sometimes present in paints as one of the constituents of a flake material referred to in the trade as "bronze" powders. So-called "gold" paint, for example, is a bronze powder made from an aluminum-copper alloy having a golden lustre. Other metal pigments containing copper are made in colors from bronze to that of copper. Even the so-called "copper-bronze" paints, however, are made from copper alloyed with other metals, principally zinc. The pigment powders for all these copper alloy paints, in common with aluminum powders, have been made in the past by the pounding of the alloy into the form of very fine flakes. Pure copper is not readily reduced to flake powder in this way and for this reason, in the past, it has been necessary to alloy it with some other metal adapted to give this property.

Copper powders have been produced in the past by electrodeposition, but such powders have consisted of minute particles of dendritic metal similar in shape to a pine tree. Also, such depositions have required special technique in the electrodeposition, such as unusually high current densities and unusually low acid and copper concentrations in the electrolyte.

An object of the present invention is to provide a process whereby pure copper may be electrolytically deposited in flake form. A further object is to provide means and a method for controlling the conditions in the electrolytic cell so that the copper will be deposited in flake form. Another object is to provide such a process by which the flake copper so deposited will be coated with an oily or greasy film.

It is also an object to provide a process for producing copper in flake-like form under the normal conditions of electrolyte composition, temperature and current density used in tank

room copper refining, and thereby to perform the operations of refining the copper and reducing it to flake form in a single step with very little additional cost of power and labor over that required for the production of ordinary cathode copper.

It is another object to produce a new product and a new procedure useful in the preparation of copper paints and other copper-containing products. Other objects will become apparent.

It has now been found that by electrolytically depositing copper upon a cathode in an electrolytic cell, which cathode is coated with a particular type of film, the copper so deposited will be in the form of an aggregate made up of individual flake-like or laminar particles instead of the usual tree-like particles and that such particles will be coated with a coating resulting from the film used. The selection of the film and the control of the oxidizing properties of the electrolyte during the electrodeposition are important in obtaining the desired results.

It has been found, for example, that a vegetable oil (or other glyceride oil or the fatty acid, or other derivative containing the fatty acid radical, corresponding to the glyceride of the oil) containing a saturated or an unsaturated hydrocarbon chain together with one or more hydroxyl groups, and having a certain degree of oxidation, 25 may be used to form the film on the cathode. The coating applied may be one that already has the required degree of oxidation or the required degree of oxidation may be obtained by controlling the oxygen content of the electrolyte.

Important characteristics of the present preferred materials forming the film on the cathode during the electrodeposition are first, that they contain fatty oils, fatty acids or derivatives of these containing the fatty acid radical, or

mixtures of two or more of these, in which there is present in the free or combined fatty acid radical, one or more hydroxyl groups, and secondly, that there must be present in the oil a definite degree of oxidation, perhaps accompanied by the formation of peroxide groups in the fatty acid radical. The coating on the cathode may also contain other substances, such as lubricating agents, or other agents useful in preparing, or for modifying the character of, the finished powder. Such other substances should be present in sufficient quantities to give the desired effect, but in insufficient quantities to deleteriously affect the electrodeposition of the flake copper.

Castor oil or the fatty acids from it are the

most important naturally occurring oil or fat containing substantial amounts of such a hydroxylated fatty acid component. Therefore, this oil or its fatty acids will be referred to in describing the invention. It is obvious, however, that other natural fatty acids or glycerides may be used or that fatty acids or fatty acid glycerides or other glycerides containing the desired hydroxyl groups may be synthesized or prepared as hereinafter indicated, or otherwise.

The oxidation of the coating material may be effected in a number of ways, for example:

1. By chemical oxidation, as by mixing the coating material with an oxidizing agent, such, for example, as a solution of hydrogen peroxide, sodium peroxide, potassium permanganate, etc. or perchloric acid or concentrated sulfuric acid, etc.

2. By blowing the coating material, before its application to the cathode, with air or other oxygen bearing or oxidizing gases or by applying the coating material to the cathode, in the form of a fine spray or by otherwise contacting it with an oxidizing gas; such oxidation is somewhat accelerated by elevated temperatures.

3. By the absorption of the coating material during the period of electrodeposition, of oxygen dissolved in or carried by the electrolyte.

The hydroxyl group may be obtained, for instance:

1. By using castor oil or mixtures of castor oil and/or its fatty acids or other natural glycerides containing at least one hydroxyl group.

2. By the hydrolysis of the peroxide or other oxidized groups formed by one of the above methods of oxidation. This hydrolysis results, for example, from the reaction of a fatty oil or other glyceride or fatty acid, having unsaturated bonds, with an acid copper sulfate solution. For instance, the hydroxyl groups may be formed in situ by the reaction between an oil or fatty acid having a high iodine number, such as a linseed oil that has been boiled with a metallic drier, with the acid copper sulfate electrolyte. This reaction goes rapidly at temperatures above 150° F. and at an appreciable rate at lower temperatures. The formation of hydroxyl groups in this way is accompanied by the destruction of some or all of the peroxide or other oxidized groups, so further oxidation may be necessary.

Thus, the control of the electrodeposition to obtain the desired result may be effected by regulating the degree of oxidation of the coating or film on which the copper deposit is to be formed. This may be accomplished by saturating the electrolyte with oxygen, for example, by splashing it into the tank, by spraying it, by dispersing or passing oxygen or an oxygen carrying gas to or through it, or by circulating it through a depositing out cell containing an insoluble anode or by other suitable means. When the control is affected in this way, the coating film on the cathode need not be pre-oxidized before the cathode is put in the electrolyte.

Or the control of the oxidation of the coating or film may be accomplished by subjecting the coating or film to a regulated pre-oxidation, either by the use of oxidizing chemicals or by exposing it to contact with oxygen or oxygen carrying or other oxidizing gases, in which event the oxidation of the electrolyte may be controlled or minimized by excluding oxygen from it and avoiding excessive splashing of the electrolyte.

Of course, regulated combinations of these two

methods for effecting control of the oxidation of the coating material or film may be utilized. For example, the coating material or film may be preliminarily chemically or otherwise treated to increase its susceptibility to oxidation, after which it may be subjected to a less intensive oxidation, either in the electrolyte or before, to obtain the desired result.

The temperature of the electrolyte may also be regulated to control the effectiveness of the oxidation of the coating material or film in the electrodeposition. For example, where there is excessive oxidation of the coating material or film, through the electrolyte or otherwise, this excessive oxidation may be compensated for to a certain extent by raising the temperature during the electrodeposition.

In describing the invention, reference will be made to an apparatus suitable for use in carrying it out, although it is not intended to limit the invention to the particular apparatus or details of procedure referred to in the description.

Figure 1 is a diagrammatic side elevation of an apparatus suitable for carrying out the process.

Figure 2 is an enlarged plan view of the electrolyte tank shown in Figure 1.

Figures 3 to 8 are photomicrographs of copper deposited in accordance with the invention.

Figure 3 is of a sectional fracture of the deposit stripped from the cathode blank, the side of the specimen at the left having been in contact with the cathode blank. Figure 4 is of the outer surface of the deposit (the right hand side of Figure 3). Both of these views were taken with vertical illumination at a magnification of 32 diameters.

Figure 5 is of powder settled dry on a glass slide with vertical illumination. Figure 6 is of particles of the powder imbedded in a resin (Pontalite), the view being taken of a section cut through the resin and through the powder suspended therein with vertical illumination. Figure 7 is like Figure 6 except that it was taken with dark field illumination. Figures 5, 6 and 7 were each taken at a magnification of 200 diameters.

Figure 8 is of particles of the powder settled dry on a glass slide. It is taken with dark field illumination at a magnification of 1000 diameters.

Referring to the drawings of the apparatus, the numeral 1 indicates an electrolytic cell having a wooden frame 2 and a lead lining 3. On the top of this tank is placed a wooden frame 4 for supporting two triangular contact bars 5 and 5a. The anode supporting bars 6 contact the triangular bar 5a at one end and rest upon the wooden frame 4 at the other end. The cathode blank carrying bars 7 rest upon the triangular bar 5 at one end and upon the other side of the wooden frame 4 at the other end. The cathode blanks are made of sheet copper, which may be riveted to the supporting bars 7. The anodes used are regular cast copper anodes. The anodes may be supported by means of copper rings 6a passing under lugs on the anodes and over the copper bars 6, which support them and provide electrical contact with the anode contact bar 5a. If desired, the cathode and anode supporting bars may be constructed and arranged so that all of the cathodes and/or all of the anodes may be immersed in and withdrawn from the cell simultaneously by means of a suitable rack and lifting cranes.

The electrolyte may be circulated through an external circuit to maintain it uniform and at the desired temperature which may be about 125 to 140° F. and preferably about 130° F. This external circuit may include a depositing out cell or other means for regulating the oxygen and other substances carried by the electrolyte. In the apparatus shown, the electrolyte flows into the cell through a glass pipe 8, leading nearly to the bottom of the cell, and flows out through the pipe 9, positioned at the opposite end and near the top of the cell, and into the lead lined wooden sump tank 10. The cell 1 may also be provided with means for separately drawing off the slimes and the liquor above the slimes, whereby the electrolyte above the slime level may be withdrawn and the slimes may be washed by means of water into a suitable receptacle. Also, if preferred, the electrolyte may be fed in near the top of tank 1 and withdrawn from near the bottom of that tank.

The electrolyte in the sump tank 10 may be pumped to a head tank 11 by means of a centrifugal pump 12 suitable for handling the acid copper sulfate electrolyte, or by other suitable means, such, for example, as an air lift pump. The head tank 11 may be provided with a heating element 13, heated by steam or electricity or other suitable means, with thermostatic control for regulating the temperature. The tank 11 may be provided with a discharge pipe 14 connected with the pipe 8 through a gooseneck 15, so that liquid can never be discharged below a definite point in the tank 11, in order to protect the heater 13 from exposure in the event an electric heater is used. Of course, when other means is provided for heating the liquid, it may be desirable to eliminate this feature. An open vent 15a is provided in the gooseneck 15 and an overflow pipe 11a, leading back to the sump tank 10, is provided so that a constant head may be maintained in the head tank 11 by circulating an excess of liquid with the pump 12.

If desired, either or both of the sump tank 10 and the head tank 11 may be provided with cathode blanks and lead sheet anodes, of the same size, for the purpose of depositing out the copper that tends to build up in the electrolyte. The oxygen liberated at the lead anodes in such an arrangement also serves to aerate the solution flowing to the electrolytic tank.

As a specific example of the carrying out of our invention in an apparatus as described above, the cathode blanks may be sprayed with hot oxidized castor oil by means of an atomizing type of spray gun. The oxidized oil may be prepared by stirring about 1% by weight of perchloric acid (about 60% perchloric acid in aqueous solution) into a good clear grade of raw castor oil (AA grade) in a kettle heated, for instance, to approximately 212° F. by steam, or other suitable means, to reduce its viscosity. The hot oil may be drawn from this kettle and sprayed as it is required. Or the cathode blanks may be dipped in the hot oil.

The oxidized oil, heated to a lower temperature if desired, may be thinned with a mixture of commercial grade denatured alcohol and enough carbon tetrachloride may be added to remove the fire hazard. The cathode blanks may then be sprayed with or dipped in this mixture and the solvents evaporated.

The degree of oxidation of the oil applied depends to a certain extent upon the tempera-

ture and the fineness of division of the particles. If the oil is sprayed with a non-atomizing type of spray gun, or if the cathode is dipped, a lesser amount of oxidation of the coating will occur than when the oil is atomized. Similarly, if the temperature is reduced, the degree of oxidation will be decreased. Variations in the degree of oxidation may be compensated for by reducing or increasing the quantity of perchloric acid used or the amount of oxygen in the electrolyte or the temperature of the electrolyte.

The cathodes prepared as described above may be placed in the electrolytic cell 1, spaced, for example, at about 4½ inches and with the anodes equally spaced between them.

A constant condition of aeration may be maintained by circulating the electrolyte, the electrolyte being, in effect, partially saturated with oxygen by allowing it to splash or by other means mechanically bringing it into contact with air.

The electrolyte may be brought up to the proper temperature (preferably no higher than 140° F. nor lower than 120° F., although satisfactory results have been obtained at higher and lower temperatures). Current may be supplied to the anodes so as to give a current density of about 15 amperes per square foot of anode surface, the corresponding cathode current density being about 15 amperes per foot. Satisfactory results may be obtained with a greater or less current density, but it is preferred to use an anode current density of about 15 to 20 amperes per square foot and a cathode current density of about 15-20 amperes per square foot.

Concentrations of copper sulfate, sulfuric acid and electrolyte impurities need be no different from the usual tank room electrolyte for electrodeposition of copper. It is advisable to maintain a chloride content of about .001 to .003% by addition of chloride compounds, for example, sodium chloride or hydrochloric acid.

With a cathode sprayed with an oxidized oil as described above, the dissolved oxygen in the tank electrolyte should be the equivalent of that present in an electrolyte through which oxygen has been bubbled to such an extent that bubbles of essentially pure oxygen will appear when a sample of the electrolyte is heated to 190° F.

The system may be maintained constant by regulating the temperature and circulation of the electrolyte and by adding or removing substances as they become depleted or excessive. After a sufficient deposit has been built up on the cathode blanks, for example, in about 24 hours, they may be withdrawn and the copper stripped from them by means of a stripping knife. The blanks may be re-oiled and returned to the cells for the next deposit.

By the procedure described, a deposit of pure copper in the form of fine laminae or flakes is produced.

Figures 3 to 8 illustrate the form of the deposit. The sectional fracture enlarged in Figure 3 illustrates the honeycomb structure of the large number of fine flakes and shows that the flakes intersect at angles of approximately 60°. Figure 4, looking at the surface of such a deposit, indicates that the multiplicity of these planes intersect to form tetrahedral pyramids, each with its apex pointing outward from the cathode blank. Figures 5, 6 and 7 further illustrate the laminar or flake-like structure. Figure 5 is a photomicrograph of the powder ob-

tained directly from the electrolytic deposit, without further treatment, except drying. In Figures 6 and 7, which are of such a powder suspended in a resin (Pontalite), both the edges of the sides of particles, may be seen clearly illustrating the flat flake-like structure. Figure 8 illustrates the fine structure of a typical flake of the electrolytic flake copper powder. Its structure consists of three sets of lines intersecting one another at angles of 60° and shows that the deposited flakes have a well defined crystalline structure. The faces of the copper flakes are sections of the (111) planes of crystalline copper. (The plane passing through the outer terminals of the three edges of a unit cube converging at a single corner of the cube, or planes parallel thereto, are 111 planes.)

This product has many uses and is particularly suited for the production of copper paints, inks, etc. The oil on the cathode blank supplies a coating of oil around the flakes of copper which expedites the subsequent wetting of the particles with the oil vehicle of the paint.

Instead of depending upon splashing or spraying to dissolve oxygen in the electrolyte or oxidize the coating composition, pure oxygen may be bubbled through the electrolyte or the coating material. Or the castor oil or other oil or substance containing the hydroxyl group may be reacted with neutral potassium permanganate, followed by washing with hydrochloric acid to decompose the manganese dioxide. Or hydrogen peroxide may be used to oxidize the oil. The oil so treated may have sulfated or Turkey red oil, for example, 1 to 5%, mixed with it.

Like amounts of 95% sulfuric acid (oil of vitriol) may be used in place of the perchloric acid referred to above.

The treatment of castor oil with sulfuric acid results in a mixture of sulfated or sulfonated castor oil and castor oil. Instead of producing the sulfonated castor oil in this way, it may be produced separately and added to the castor oil, or Turkey red oil, which is a sulfated castor oil neutralized to destroy excess acid, may be added to the castor oil. The desired percentage of sulfonated or sulfated castor oil, or Turkey red oil, varies with the oxygen content of the electrolyte and with the degree of oxidation of the castor oil. The greater the oxygen content or degree of oxidation of the castor oil, the smaller is the quantity of sulfonated castor oil or Turkey red oil that should be used in the mixture. Satisfactory results may be obtained in the electrodeposition described above when a castor oil treated with 1% of sulfuric acid is sprayed with an atomizing spray gun onto the cathode blank and the oxygen content of the electrolyte is equal to that of an electrolyte in which bubbles of pure oxygen would start to be liberated at a temperature of about 190° F.

Satisfactory results have been obtained using about 4 1/2 to 5% by weight of sulfated castor oil or Turkey red oil in castor oil, with electrolyte temperatures of about 122 to 157° F. and circulating with an air lift pump whereby a condition of intensive electrolytic aeration was obtained.

Good results have also been obtained by saponifying castor oil with 25% of sodium peroxide and a minimum of water, the mixture being heated to 212° F. and cooled and acidified. This oil was diluted with 5 times its weight of raw grade AA castor oil and sprayed on the cathode. The electrolyte temperature was maintained at

about 121 to 126° F. and the electrolyte aeration was minimized by eliminating all splashing from discharge pipes. This run lasted for 68 hours.

Good results have also been obtained by spraying the cathode with mixtures of castor oil and linseed oil. For example, excellent deposits were obtained with a mixture of 75% linseed oil and 25% castor oil, slight aeration being maintained by allowing the discharge liquor from the pump to splash upon the surface of the electrolyte in the head tank. The temperatures were maintained at about 128 to 143° F. With moderate aeration excellent powder was obtained with such a mixture at temperatures of 133 to 137° F. The temperature of spraying the oil onto the cathode was varied from 100 to 180° C. without observable difference.

Good flakes were also obtained using castor oil treated with .5 to 2.5% of perchloric acid (60%). The perchloric acid was stirred into the castor oil (grade AA) until an emulsion was formed at room temperature. The emulsion was then heated to 90 to 100° C. until it was changed to a clear, slightly brown colored solution, which was sprayed onto the cathode. The temperature was maintained at 126 to 130° F. and electrolyte aeration was minimized. In these tests very good flake deposits were obtained in runs lasting for 22 to 47 hours.

Good results were also obtained by treating the castor oil to be applied to the cathode with perchloric acid (60%) or sulfuric acid (95%) as hereinbefore described, and controlling the oxidation of the electrolyte by passing gaseous oxygen through the electrolyte in the head tank, the said gaseous oxygen being diffused through a porous thimble in the bottom of the tank. The oxygen content of the electrolyte was measured by heating a portion of the electrolyte very gradually and noting the temperature at which bubbles of essentially pure oxygen appeared.

Good deposits were obtained by following this procedure and using percentages of sulfuric acid from about 2.5 to 1% at electrodepositing temperatures of about 124 to 131° F., the oxygen content being such that bubbles of oxygen appeared in portions of the electrolyte that were heated to about 170 to 192° F. A fair deposit was obtained with .1% sulfuric acid at an electrolyte temperature of about 128° F. and with oxygen bubbles appearing at about 184° F.

Similar results were obtained with castor oils treated with perchloric acid (60%) in the amounts given above and at the same range of electrolyte temperatures, the oxygen content of the electrolyte being such that the bubbles of oxygen appeared on heating the electrolyte at the same range of temperatures. Oxidation with perchloric acid appeared to give better results than the oxidation with sulfuric acid, inasmuch as the deposits were more uniform and the flakes were finer. Also, it was less sensitive to changes in the amount of oxidizing agent used and the degree of oxidation of the electrolyte than with sulfuric acid. With mixtures of sulfuric and perchloric acids, the results obtained were intermediate between those obtained with the two constituents separately.

It has been found that with proper oxidation the temperature of the electrolyte may vary between 120 and 145° without affecting the deposit a great deal, except that at the higher temperatures the viscosity of the oil is reduced to a point at which it tends to rise along the blank, becoming thin at the bottom and heavier at the top,

so that the deposit is of an uneven character. Satisfactory results were also obtained with temperatures outside of this range for a portion of the electrodeposition period. It was found desirable to maintain the chlorine content of the electrolyte at about .001%. This may be accomplished by adding hydrochloric acid or salt, etc.

Electrolytes that analyzed 14 to 20% free H<sub>2</sub>SO<sub>4</sub>, 2.4 to 4% copper and .001% to .004% of chlorine have been found to be satisfactory. It is preferred to maintain the electrolyte within the range 16 to 18% free H<sub>2</sub>SO<sub>4</sub>, 3 to 3.5% Cu and .0015 to .003% Cl.

Satisfactory deposits have also been obtained with boiled linseed oil containing a lead drier and with mixtures of Turkey red oil with various fatty acids.

From a practical consideration it is desirable to operate so as to obtain a satisfactory deposit for the longest possible period. As the length of the run increases the percentage of coarse flakes decreases. Generally speaking, when the product is required to be such that after the initial disintegration and flotation 85 to 90% of the metal will pass through an 80 mesh sieve, the run should be limited to about 24 hours. This period may be lengthened by more accurate control of the conditions in the cell during the electrodeposition. If there is a larger measure of tolerance the run may be extended up to 72 hours or more. To lengthen the run the oxygen contained in the electrolyte or the degree of oxidation of the oil or the susceptibility of the oil to oxidation should be slightly decreased. Too much oxidation tends to shorten the period before the deposit becomes tough and flakes are no longer deposited. On the other hand, too little oxygen tends to cause the initial deposit formed to be coarse and possibly tough, but after a time the flakes deposited will become finer and better. In order to avoid coarse particles in the powder, it is desirable to keep this induction period as short as possible.

Although it is not intended to limit the invention to any particular theory of operation, it is believed that the oil or other coating material accomplishes its function by stopping or strongly retarding the component of crystal growth in either direction perpendicular to one of the (111) planes and to allow growth to proceed in the (111) plane. Thus the growth may proceed freely along the face of the plane but to only a restricted degree along a perpendicular to this plane. The function of the oil or other coating is to selectively wet the deposited copper so as to limit the component of its growth perpendicular to the (111) plane. Thus by wetting the (111) planes of the copper crystal lattice far more effectively than any other plane, the component of growth perpendicular to this plane is inhibited while the growth is permitted to proceed parallel to or along this plane, resulting in a laminar crystal.

Three factors are important in their effect upon the orientation of the molecules of oil or other coating material: (1) the attraction (wetting) holding one part of the molecule to the face of a copper crystal; (2) the effect of the electric field, which is perpendicular to the cathode surface; and (3) the orienting effect of the attractive and repellent forces of neighboring molecules.

The first of these must be present if the oil is to wet the copper at all, which apparently is essential to the formation of flake deposits.

Also, if the wetting power is too great, the crystal growth may be hindered parallel to as well as perpendicular to the (111) plane. The strength of wetting is determined, in the case of fatty acids and their glycerides, by the degree of oxidation imparted or obtained.

The second factor is responsible for the orientation of the flakes symmetrically about lines perpendicular to the cathode (see Figure 3).

The third factor affects the nature and sizes of the individual flakes. If the oil molecules on the surface of the copper are strongly attracted or associated, and if their configuration is such that they may properly align themselves, they will tend to be well oriented and the laminar crystals will grow in area very considerably before interruption occurs, leading to crystallization in another of the four possible directions. When the interruptions are relatively few, the individual flakes grow quite large and the deposit is very bulky. On the other hand, when they are numerous, the individual flakes are smaller and the deposit more compact. Hydroxyl and peroxide groups favor association and hence this type of molecular orientation. For the best molecular orientation it is desirable that the molecules have essentially a chain structure.

Although we have given a number of specific examples of coating materials suitable for accomplishing the desired result, it is not intended to limit the invention to these, since it will be apparent that other substances that will selectively inhibit or retard the growth of the crystals in various directions, may be used in place of the illustrative examples.

The aggregate of flakes stripped from the cathodes in following the above described procedures may be washed by means of any suitable washing device. The washings may be returned to the tank electrolyte, if desired. For instance, the flakes may be covered with water and allowed to soak for a day, after which the supernatant liquor may be returned as make-up water to the sump tank. The remaining flakes may be dumped into the agitator in which it may be allowed to remain until the time at which it is desired to operate the flotation cell.

The contents of the agitator may be agitated by an impeller, which serves to disintegrate the agglomerated lumps of flakes of copper, and discharged into the flotation cell. The flotation cell may be of the usual type provided with an impeller. It is preferred to use a cell of the sub-aeration type; i. e., one with an impeller and an air inlet under the impeller. The oil films on the particles of copper, resulting from the oil applied to the cathode blank, provides a flotation agent so the flotation cell may be operated without any reagents other than the oil already present on the copper flakes.

If desired, the disintegration and flotation may both be accomplished in the flotation cell by providing a suitable impeller therein.

A classification of the particles is achieved in the flotation cell, the coarse lumps being allowed to collect in the bottom of the machine. The fine froth may be discharged by means of a scraper and may be de-watered in a centrifuge or other suitable water separating device, such, for example, as a continuous rotary filter. Hot water may be used in washing the flakes during this operation.

The cake from the centrifuge or rotary filter contains approximately 20% water which may be removed in a drier, operated at a temperature

of not higher than 550° F. The atmosphere in the drier should be inert, containing such gases as carbon dioxide, nitrogen, etc. Where a rotary kiln type of drier is used, a continuous rotary filter may be used, while if a batch drier is used, a centrifugal separator may be preferable. The drying may be suitably accomplished by heating with steam heat while applying a suction. In order to avoid the possibility of oxidation, the air in the drier may be displaced with carbon dioxide or other inert gas before the application of heat and vacuum and the inert gas may also be allowed to bleed into the drier during the first few hours of the drying operation. After the drying, cooling water may be passed 15 through the heating unit to cool the flakes and after cooling the vacuum may be broken and the flakes removed.

The material discharged from the drier may be disintegrated in a ball mill, etc., to prepare it 20 for use in the production of paints, inks, etc. or for other desired uses. In such preparation, it is preferred to avoid oxidation of the copper powder and the disintegration is preferably carried out in the absence of oxygen by displacing 25 the air in the mill with carbon dioxide or some other inert gas before the grinding. Also, in the preparation of flake copper for use in paints, etc., it may be desirable to avoid leafing or mirroring of the flakes. Such leafing or mirroring cause 30 the particles of copper to float to the surface of the paint, etc. vehicle and remain there after drying of the film, with the result that the copper is exposed to the atmosphere and will tarnish easily. For some uses it is preferred to prepare 35 the flakes in such a manner that it will be completely dispersed and distributed throughout the body of the film, so that the particles will be protected from the atmosphere.

Various solvents, vehicles, resins, etc., useful 40 in the preparation of paints, etc., may be added to the copper flakes before or after the disintegration of the dried product. It is desirable that the vehicle used be quick setting in order that the coagulation or settling of the metal flakes 45 during the period of drying will be avoided. A good dispersion of the pigment is relied upon to obtain the desired high covering power and dispersity. An example of a vehicle which meets the requirements specified above is a short or medium oil alkyd resin containing about 35% of the film forming ingredient in solution in a toluol-xylol thinner and having a viscosity of 2 to 2½ poises. The relatively high viscosity serves to aid 50 the dispersion of the flakes and to avoid leafing. An example of an entirely different type of vehicle, equally successful, is a varnish made from Tornesit (a chlorinated rubber compound), plasticized with Arochlor (a chlorinated biphenyl), which may be dissolved in a mixture of xylol and hydrogenated petroleum thinner. The number of other materials which may be used is large.

The percentages referred to in this application are by weight.

It is obvious that many variations may be made in the procedures described for depositing the aggregate and for preparing it for various uses and it is not intended to limit the invention to the particular examples and illustrations given.

The terms used in describing the invention have been used in their descriptive sense and not as terms of limitation and it is intended that all equivalents thereof be included within the scope of the appended claims.

We claim:

1. A method for preparing metallic copper in fine flake form comprising electrodepositing copper, from an aqueous acid solution of a copper compound, upon a cathode carrying a composition containing an oxidized fatty acid radical having at least one hydroxyl group.

2. A method for preparing metallic copper in fine flake form comprising electrodepositing copper, from an aqueous acid solution of a copper compound, upon a cathode carrying a composition containing an oxidized fatty acid oil having at least one hydroxyl group in the fatty acid radical.

3. A method for preparing metallic copper in fine flake form comprising electrodepositing copper, from an aqueous acid solution of a copper compound, upon a cathode coated with a composition containing an oxidized castor oil.

4. A method for preparing metallic copper in fine flake form comprising electrodepositing copper from an aqueous acid solution of a copper salt upon a cathode carrying a composition that is a flotation collecting agent and that contains an oxidized fatty acid radical having at least one hydroxyl group, stripping the copper from the cathode, churning it into a fine froth and separating the fraction containing the fine particles.

5. A method for preparing metallic copper in fine flake form comprising electrodepositing copper, from an aqueous acid solution of a copper compound, upon a cathode carrying a composition that is a flotation collecting agent and that contains an oxidized fatty acid radical having at least one hydroxyl group, stripping the copper from the cathode, washing it, churning it into a fine froth, separating the fraction containing the fine particles and drying the fine particles in an inert atmosphere.

6. A method for preparing copper in fine flake form, which comprises electrolytically depositing the copper from an aqueous acid solution of a copper salt upon a cathode face coated with a composition containing an oxidized fatty acid radical having at least one hydroxyl group, which causes the deposition of an aggregate of laminar crystals and coats these crystals with a flotation collecting agent, stripping the aggregate of crystals from the cathode face, churning the mass into a fine froth wherein the said coating material serves as a flotation collecting agent, and separating the fraction containing the fine particles by froth flotation.

7. A method for preparing flake copper, comprising electrodepositing copper from an aqueous acid solution of a copper salt upon a cathode carrying a composition containing an oxidized fatty acid radical having at least one hydroxyl group, stripping the copper from the cathode, washing it free of electrolyte, and drying it at a high temperature.

8. An article of manufacture comprising a pure metallic copper electrodeposited in flake form and having thereon a film of an oily composition containing an oxidized fatty acid radical having at least one hydroxyl group, said flake copper being electrodeposited from a cathode coated with said oily composition.

9. An article of manufacture comprising electrodeposited flakes of copper, the faces of which correspond to (111) planes of the crystal lattice, said flakes being coated with an oily or greasy material containing an oxidized fatty acid radical having at least one hydroxyl group and

being electrodeposited from a cathode coated with said oily or greasy material.

10. An article of manufacture comprising a pure metallic copper electrodeposited in flake form from a cathode coated with an oily composition containing an oxidized fatty acid radical having at least one hydroxyl group, said flake copper as deposited having a film of oily substance derived from the cathode thereon.

11. A method of preparing metallic copper in fine flake form, comprising electrodepositing copper from an aqueous acid solution of a copper compound, at temperatures of 120 to 140° F.,

upon a cathode carrying a composition containing an oxidized fatty acid radical having at least one hydroxyl group.

12. A method of preparing metallic copper in fine flake form, comprising electrodepositing copper from an aqueous acid solution of a copper compound, at temperatures of 120 to 140° F., and current densities of 15 to 20 amperes per square foot, upon a cathode carrying a composition containing an oxidized fatty acid radical having at least one hydroxyl group.

SIDNEY B. TUWINER.  
WILLIAM H. OSBORN.